

April 13, 1937.

C. F. LAUENSTEIN

2,077,117

FERROUS ALLOY AND PROCESS OF PRODUCING FERROUS ALLOY

Original Filed April 7, 1933

Fig. 1.



Fig. 2.



Inventor  
Carl F. Lauenstein  
by Parker & Carter  
Attorneys.

## UNITED STATES PATENT OFFICE

2,077,117

FERROUS ALLOY AND PROCESS OF PRO-  
DUCING FERROUS ALLOYCarl F. Lauenstein, Indianapolis, Ind., assignor to  
Link-Belt Company, Chicago, Ill., a corporation  
of IllinoisOriginal application April 7, 1933, Serial No.  
664,902. Divided and this application Decem-  
ber 13, 1934, Serial No. 757,290

## 6 Claims. (Cl. 148—21.8)

This application is a division of my co-pending application Serial Number 664,902, filed April 7, 1933, which is itself a continuation in part of my application Serial Number 475,829, filed August 6, 5 1930.

This invention relates to a ferrous alloy and to the process of producing it. The raw material from which the metal is produced is essentially malleableized cast iron which contains certain 10 strengthening alloying elements. Among those which may be used are nickel, molybdenum and copper, manganese, chromium, vanadium and aluminum. These may be used in varying amounts.

15 As generally understood, ordinary malleableized cast iron is granular in its structure, being composed mainly of grains of ferrite and small particles of carbon or graphitic carbon. One step in the present method or process is designed to cause a combination of the carbon and the ferrite 20 in order to form pearlite or iron carbide.

Another object is to produce a metal and a process for making it in which the metal is stronger than ordinary malleableized cast iron and stronger 25 than ordinary malleableized cast iron after it has been treated by my heating process. The presence of the alloying elements in the metal improves the physical properties, particularly improving the ultimate strength, the yield point and 30 the elongation.

Other objects will appear from time to time in the specification and claims.

The metal of the present invention is formed from white cast iron. Before the commencement 35 of my process the iron is put through any standard or suitable malleableizing process. White cast iron has an average chemical composition as follows:

|                  | Percent   |
|------------------|-----------|
| Combined carbon  | 2.30-2.40 |
| Graphitic carbon | Nil       |
| Silicon          | .90-.95   |
| Manganese        | .27       |
| Sulphur          | .060      |
| Phosphorus       | .16       |

To this may be added suitable quantities of copper, molybdenum, nickel, manganese, chromium, vanadium, aluminum or other alloying elements. These alloying elements may be added 50 into the cast iron in the furnace or the ladle, or at any time before the iron is finally molded. The white cast iron with the alloying elements is poured into suitable molds and allowed to cool. It may then be cleaned and after cleaning it is 55 put through any suitable malleableizing process.

After the malleableizing process is completed a subsequent heat treatment is applied to the metal. This heating will usually be done in furnaces, but may, of course, be done by any other means. The iron is raised to a temperature between 1375° F. and 1500° F. This temperature is given as approximating the best temperature, but a variation either above or below this temperature is possible. After the material has reached the critical or carbon combining temperature a part of the carbon is combined with ferrite. The length of time that the material being treated must be held at this temperature varies with the size of the parts being treated and with the physical properties desired. After the heating has been carried on a sufficient time, the parts are then quenched, that is to say, cooled, in air, oil, water or other medium. In ordinary practice, no particular effort is made to cool the metal slowly and where it is quenched in oil or a liquid, it is usually cooled rapidly. Where it is desired to give the metal a tough and wear resisting outer coat, the heating operation will be carried out in the presence of a carburizing agent.

When the material being treated has been first heated and quenched, it is thereafter reheated to a temperature not exceeding the critical or carbon combining temperature. The result of this second heating is to cause the martensite or troostite retained after the first heating to break down into pearlite or sorbite. This change will normally be effected at a temperature range of 900° F. to 1350° F. The cooling, after the second heating, is preferably air cooling although a water or oil quenching may be used, depending somewhat upon the physical properties desired. A water quenching produces a stiffer, higher strength iron, while oil and air cooling produces relatively more ductile iron. Any cooling method may be used.

The accompanying drawing illustrates in Figure 1 the structural arrangement and constituents of a sample of malleableized cast iron and in Figure 2 a sample of the metal of my invention. The figures are diagrammatic showings based upon microphotographs of samples of metals. They suggest diagrammatically only typical forms of the metal. Other samples would show the same general characteristics, but would show detailed modifications.

In Figure 1 the metal is seen to be generally granular. It is composed of grains, A, which are ferrite and separated from each other along boundaries B. The grains may be of irregular shapes and sizes. Interspersed through the mass

5  
10  
1520  
25  
3035  
40  
45

50

55

of the metal are spots of free or graphitic carbon C.

Figure 2 is a diagram based upon a microphotograph of a section of a sample of the metal of this 5 invention.

As illustrate in the drawing, the metal is generally granular, being formed of grains A. These grains are bounded or separated along boundaries B. The grains are in the form of 10 ferrite. C represents a spot of graphitic or free carbon. In a larger sample of the metal a number of such spots of graphitic carbon would appear. Situated throughout the metal, surrounding the grains and the graphitic carbon and filling the great majority of the grain boundaries and to some degree penetrating within the ferrite grains themselves is pearlite. This material is 15 indicated at D.

Figure 2 illustrates an important characteristic 20 of the present invention, namely that there is distributed throughout the metal, along the grain boundaries and about such particles of graphitic carbon as are present, an agent which tends to stiffen the grains and prevent their 25 distortion under stress, thus strengthening the mass and preventing the separation or pulling apart of the grains. This agent is an iron carbide with alloy content and in the form illustrated in Figure 2, is normally pearlite or sorbite. It 30 is characteristic of this iron carbide, which in this case may be pearlite or sorbite, that it is strong and tough and it thus strengthens the grains against distortion, holding the grains together more strongly than in other cast iron 35 where the ferrite is combined without the presence of any appreciable amounts of alloy pearlite at the grain boundaries. It thus increases the tensile properties of the material.

It also makes the metal of the invention 40 highly resistant to wear or abrasion. The harder and tougher alloy pearlite or alloy sorbite at the ferrite-grain boundaries acts as a guard preventing the wearing or abrading away of the softer ferrite grains. The pearlite or sorbite is 45 strengthened by the alloying element.

In the metal of this invention, the main body 50 of the metal is made up of a group of ferrite grains. The great majority of these grains is surrounded each with a harder shell of pearlite or sorbite, that is to say, with a shell of an iron carbide with alloy content which has such physical properties that it tends to strengthen the grains of ferrite. It prevents deformation of the grain and by this fact it resists distortion 55 of the grain and resists breaking of the grain itself or separation of one grain from the other. This iron carbide in the body of the metal may be said to act like an iron reinforcement about a piece of wood. It prevents distortion and so 60 prevents splitting and breaking. Thus in the metal of this invention there is built up throughout the body of the metal a reinforcing framework of the stronger iron carbide which has many cell-like compartments in it. These cells 65 surround the weaker grains of the ferrite which are thus strengthened and the separation of these grains of ferrite is resisted by this cell like structure of the carbide. In effect there is 70 built up a structure which may be likened to a honey comb. This is formed of the iron carbide and within the cells of the honey comb are found the grains of ferrite. The honey comb thus serves to strengthen the individual grains and 75 to resist deformation of them and further, to re-

sist deformation of the mass as a whole and to prevent separation of the grains.

As above indicated, the metal owes its strength to the presence of the pearlite or iron carbide network surrounding the grains and lying within and along the grain boundaries. The presence of the alloying metal gives this network a higher strength and hardness than that which it would otherwise have if the alloying element were not present.

The temperature ranges above suggested are 10 not absolute limits and are indicated for the first heating as being within the range of the critical or carbon combining temperature, and for the second heating as being above the range of customary hot galvanizing. In the first heating the 15 temperature may be as high as 1500° F. and in the second heating it may be as low as 900° F., although in normal practice the first heating is preferably between 1425° F. and 1450° F. and the second heating is preferably between 1200° 20 F. and 1250° F.

The increased strength of my metal resultant 25 from the use of the alloying element is possibly caused by the pearlite or sorbite, including such an alloy content, having higher physical properties than pearlite or sorbite without this alloy content. This higher strength pearlite or sorbite formed at the grain boundaries has a greater stiffening effect on the ferrite grains and better resists their deformation under 30 stress, thus producing a higher strength metal. Since the physical properties of this alloy pearlite or sorbite network can be varied by different heat treatments and by the use of different alloys or different combinations of alloys, 35 the resultant properties of my metal can also be so varied.

The alloying materials above mentioned are only given as typical metals for this use. Many others might be used. For some purposes one 40 will be used alone and for other purposes two or more will be used together. Thus one alloy might include 1.50% nickel only. Other alloys might include .30% copper and .30% molybdenum and still other alloys might include .30% 45 molybdenum and 1.50% nickel. Thus a very wide variety of alloying elements and combinations of these elements may be used in my invention.

In general, the typical alloying elements and 50 the quantities of them which are most likely to be used are as follows:

|                 | Percent     |
|-----------------|-------------|
| Copper.....     | .35 to 1.00 |
| Manganese.....  | .50 to 1.00 |
| Molybdenum..... | .20 to .60  |
| Nickel.....     | .50 to 1.50 |
| Chromium.....   | .10 to .60  |
| Vanadium.....   | .10 to .60  |
| Aluminum.....   | .10 to 1.00 |

Where in the claims I have used the expression "an alloying element of the carbide forming group of elements consisting of manganese, molybdenum, chromium and vanadium", and the further expression "an alloying element of the ferrite alloying group of elements, consisting of nickel, copper and aluminum", I mean any one or more of the elements above mentioned, that is to say, molybdenum, nickel, copper, manganese, vanadium, chromium and aluminum, used substantially within the limits above stated. These alloys may be used singly, generally within the ranges indicated, or in any combination of two or more of them.

When the alloying metals are used the annealing or malleableizing cycle is generally the same as that typical of the manufacture of malleable iron. In some cases the alloy content may necessitate slight variations from the standard. One typical annealing cycle may be as follows: Heat the metal to 1650° F., this heating occupying about 36 hours; hold the metal at 1650° F. for 36 hours. Cool to 1200° F. at 6° F. per hour, occupying about 72 hours. The furnace may then be unloaded and after cooling and inspection the castings or other metal articles may be put through the secondary heat treating cycle. A typical heat treatment for metal of about .30% copper and .30% molybdenum content would be: Heat to 1475° F.; quench in oil; reheat to 1200° F. and quench in water. If the metal were an alloy including 1.00 nickel and .30% molybdenum, the first heating would be carried out to a temperature between 1400° F. and 1450° F. and the second heating would be carried out to a temperature between 1200° F. and 1250° F., and instead of the final quenching in water, the articles might be cooled by air. Other changes in temperatures and times of heating may be desirable or may be necessary where other alloying metals are used or where they are used in different proportions. Generally where nickel, copper or aluminum are used as alloying agents the first treating temperature of the heat treatment will, as a rule, be lower than 1475° F. and it may be lowered to 1400° F., due to the depressing effect that these elements have on the critical temperature. Some of the other elements listed do not have such a marked effect on the critical temperature but in general tend to raise it slightly.

It is therefore possible to use such an alloy as nickel, which depresses the critical temperature, and add to it molybdenum, which has a slightly opposite or cancelling effect, and use a first treating temperature of 1450° F. In any event, the treating temperatures must be governed by the alloying elements and the desired physical properties in the finished part.

The following analyses are given as typical of one alloy combination of metal produced by the method of this invention:

Before annealing or malleableizing treatment—

|                  | Percent |
|------------------|---------|
| Combined carbon  | 2.40    |
| Graphitic carbon | Nil     |
| Silicon          | .95     |
| Manganese        | .27     |
| Sulphur          | .060    |
| Phosphorus       | .16     |
| Nickel           | 1.50    |
| Molybdenum       | .30     |

After annealing or malleableizing treatment—

|                  |      |
|------------------|------|
| Combined carbon  | .0   |
| Graphitic carbon | 1.80 |
| Silicon          | .90  |
| Manganese        | .27  |
| Sulphur          | .060 |
| Phosphorus       | .16  |
| Nickel           | 1.50 |
| Molybdenum       | .30  |

After final heat treatment the analysis is:

|                  |      |
|------------------|------|
| Combined carbon  | .40  |
| Graphitic carbon | 1.40 |
| Silicon          | .90  |
| Manganese        | .27  |
| Sulphur          | .060 |

|            |      |
|------------|------|
| Phosphorus | .16  |
| Nickel     | 1.50 |
| Molybdenum | .30  |

The analyses given are typical of only one of a large number of possible combinations and the invention is not in any way limited to the analyses given.

Other alloys which have proved satisfactory and which include a metal of the ferrite alloying group and the carbide forming group, include the following proportions of copper and molybdenum:

|                    |                    |
|--------------------|--------------------|
| Copper molybdenum— | .30% Cu.—.30% Mo.  |
|                    | .80% Cu.—.30% Mo.  |
|                    | 1.20% Cu.—.10% Mo. |

With this alloy in the proportions indicated, it is preferable to reduce the first heating so that it is carried out to a temperature of from 1425° F. to 1475° F.

Another alloy including metal of each group is 20 nickel, 1.00 per cent, molybdenum .30 per cent.

In this alloy the first heating is preferably in the neighborhood of 1425° F. and the second heating is higher than in the general practice above suggested, namely, 1325° F.

The alloys and temperatures above indicated are merely illustrative of the fact that a wide range of modifications and combinations of alloys is possible and that for some of them it is necessary to change the heating temperatures from 30 those which are satisfactory where the metal contains no additional alloying element of the ferrite alloying group or of the carbide forming group. The invention is not limited to the particular combinations, to the particular proportions 35 or to the particular temperatures given.

I claim:

1. A granular ferrous metal, including at least one alloying element of the carbide forming group of elements consisting of manganese, 40 molybdenum, chromium and vanadium, in approximately the following proportions: Manganese .50 to 1.00 per cent; molybdenum .20 to .60 per cent; chromium .10 to .60 per cent and vanadium .10 to .60 per cent, together with at least one 45 element of the ferrite alloying group of elements, consisting of nickel, copper and aluminum in proportions up to 1.50 per cent, and including ferrite, graphitic carbon and iron carbide, the latter being distributed along the grain boundaries and 50 between the grain of ferrite and about the graphitic carbon.

2. A granular ferrous metal including an alloying element comprising: manganese .50 per cent to 1.00 per cent, and a second alloying element 55 comprising: nickel .50 to 1.50 per cent, and including ferrite, graphitic carbon and iron carbide, the latter being distributed along the grain boundaries and between the grains of ferrite and about the graphitic carbon.

3. A granular ferrous metal including an alloying element comprising: molybdenum .20 per cent to .60 per cent, and a second alloying element, nickel .50 to 1.50 per cent, and including 65 ferrite, graphitic carbon and iron carbide, the latter being distributed along the grain boundaries and between the grains of ferrite and about the graphitic carbon.

4. A granular ferrous metal including an alloying element comprising: molybdenum .30 per cent, and a second alloying element comprising: nickel 70 1.00 per cent, and including ferrite, graphitic carbon and iron carbide, the latter being distributed along the grain boundaries and be- 75

tween the grains of ferrite and about the graphitic carbon.

5. A granular ferrous metal, including at least one alloying element of the carbide forming group of elements consisting of manganese, molybdenum, chromium and vanadium, in approximately the following proportions: manganese .50 to 1.0 per cent; molybdenum .20 to .60 per cent; chromium .10 to .60 per cent and vanadium .10 to .60 per cent, together with at least one element of the ferrite alloying group of elements, consisting of nickel, copper and aluminum in the following approximate proportions: nickel .50 to 1.50 per cent; copper .35 to 1.00 per cent and aluminum .10 to 1.00 per cent, and including grains of ferrite, graphitic carbon and iron carbide, the latter being distributed along the grain boundaries and between the grains of ferrite and about the graphitic carbon.

6. The process of heat treating malleableized cast iron, which iron includes an alloying element of the carbide forming group of elements consisting of manganese, molybdenum, chromium and vanadium in approximately the following 5 proportions: manganese .50 to 1.0 per cent; molybdenum .20 to .60 per cent; chromium .10 to .60 per cent and vanadium .10 to .60 per cent and including ferrite, together with an element of the ferrite alloying group of elements consisting of nickel, copper and aluminum, in approximately the following proportions: nickel .50 to 1.50 per cent; copper .35 to 1.00 per cent and aluminum .10 to 1.00 per cent, which process includes heating the iron to a point between 1375° 15 F. and 1500° F., quenching and reheating to a point between 900° F. and 1350° F.

CARL F. LAUENSTEIN.